

Sept. 3, 1968

L. EIGENMANN

3,399,607

ROADWAY SURFACE MARKING, AND MARKED ROAD

Filed Oct. 25, 1966



INVENTOR.  
Ludwig Eigenmann

BY

Michael J. Stricker  
Attorney

**1**

3,399,607

**ROADWAY SURFACE MARKING, AND  
MARKED ROAD**Ludwig Eigenmann, % Cicogna Franco & Co.,  
14/A Via Visconti di Modrone, Milan, ItalyContinuation-in-part of application Ser. No. 262,658,  
Mar. 4, 1963. This application Oct. 25, 1966, Ser.  
No. 589,288Claims priority, application Switzerland, Apr. 13, 1962,  
4,604/62

5 Claims. (Cl. 94—1.5)

This application is a continuation-in-part of application Ser. No. 262,658 filed Mar. 4, 1963.

This invention relates to the art of marking surfaces subject to mark-obliterating traffic, and more particularly to the marking of traffic lines and other directional data upon the pavement on streets and highways, by applying on and securing road marking tape material to said pavement.

Roadmarks consisting of tape or strip materials are well known in the art, as being very advantageous in respect with conventional traffic aids, such as road-center lines, which are customarily painted upon the street or highway pavements with ordinary paints. The road-marking strip material is capable of resisting to the most severe traffic and its application to street and highway conventional surfaces requires little or no interruption to traffic. Such application can advantageously be made by making use of mechanical aids, such as the apparatus described and shown in my prior Patent No. 3,007,838.

The very scope of road marking is obviously to provide on the street or highway pavements signs and traffic data which have high daytime and nighttime visibility to motorists. Road-marking strip or tape materials as above considered can be compounded to provide traffic indicative high visibility surface portions on the marked road. The concept of "high visibility" is to be intended in its broadest meaning and cannot be defined—as far as the invention is concerned—in terms of brilliance and expressed by numerical values. Such traffic aids cannot be compared with a source of radiant energy, and are capable of reflecting ambient light only. Therefore, a "high visibility" surface portion, within the scope of this invention, will hereinafter be termed "high light reflectivity" surface portion.

The character of "high reflectivity" is however at its turn difficult to define as, according to scope of the invention, an efficiently marked road is a road having a roadway surface and traffic regulating signs located thereon, said signs being such to be distinctly and clearly seen and neatly evidenced at distance by motorists, under the most different conditions of illumination. Many variables are involved in the visibility of road markings and of traffic conditions in general. The traffic occurs under bright sun light and in rainy weather and dim ambient light, and at nighttime the roadway surface can be illuminated by powerful vehicle headlamps or by rather weak streetlamps, and therefore both intensity and direction of incident light are subject to the most wide variations.

As a matter of fact, one means for defining the visibility of a road marking or, more properly, the visibility of a traffic aid of the type considered on a roadway surface, is to compare the apparent brilliance of the road marking material considered, in several daytime and nighttime limit conditions, with the apparent brilliance of an identically shaped and positioned surface portion of a material of well known and measured reflectivity of visible light. A smooth surface of a layer of pure baryta (BaO) white may be assumed as a suitable basis of comparison. A road marking can be considered to have "high reflectivity" when, as photometrically compared as above with a simi-

**2**

larly shaped, located and illuminated sign of pure baryta, it is proved to have at least sixty percent apparent brilliance of said basis of comparison.

Therefore, the expression "high reflectivity," anywhere 5 hereinafter indicated as this description proceeds and in the appended claims, is intended to refer to a surface portion which, when photometrically compared with a surface portion of pure baryta white, it averages at least 60 percent apparent brilliance of its basis of comparison.

It has however been found that a marking tape material having the above or desirably better high reflectivity property does not possess the most desirable "non-skid" 10 properties for ensuring the most desirable safe movement and control of fastly running vehicles, in particular when 15 subject to intense positive or negative accelerations and/or to centrifugal force. It is assumed that a roadway surface portion is "non-skid" when its adherence coefficient, with respect to current tired vehicles, averages the value of 40°, in terms of angle to the horizontal at which a force cor- 20 responding to the weight applied to loaded tired wheel is directed to cause skidding of said wheel along the surface under test. The concepts of adherence offered by roadway surfaces and the modes for measuring same are well known in the art of roadway engineering and no further 25 discussion is necessary thereabout.

It is therefore an object of this invention to provide a marked road which comprises a conventional surface for vehicles and a traffic aid consisting of tape material having both high light reflectivity and non-skid properties.

According to the invention, there is provided, on a conventional roadway surface, a compound tape material 30 consisting of a first base strip having relatively non-skid properties and high light reflectivity, said base strip being adhesively adherent to said roadway surface, and strip 35 components formed of a material having lesser light reflectivity than said first strip and non-skid properties, said strip components being aligned in longitudinal direction of the first strip and are adherent thereto equally spaced from the lateral edges of the first strip, whereby, on the 40 surface of the road, a composite marking strip is formed having exposed portions formed by the first strip and having high light reflectivity and exposed center portions having non-skid properties.

By thus providing the strip with distinct portions of 45 high light reflectivity and respectively of non-skid character, the well known disadvantages and limitations of conventional marked road are eliminated, inasmuch as the marked road according to the present invention will, in its marked surface portion, possess the most desirable 50 high light reflectivity as well as higher non-skid properties than could be obtained up to now in combination with the desired degree of light reflectivity.

According to one embodiment of this invention, a strip 55 formed of a material having non-skid properties and having a lesser width than said first high light reflective base strip is extended in longitudinal direction and adhered to said base strip equally spaced from the lateral edges thereof so as to provide a composite surface formed of two spaced edge portions of said first strip having high 60 light reflectivity and of a center portion having non-skid properties and a lesser light reflectivity interposed between said two spaced edge portions of said first strip.

According to a modified embodiment of this invention, strip elements made of said material having non-skid 65 properties are adhered to said base strip equally spaced from the lateral edges thereof and evenly spaced from each other in longitudinal direction.

It has been surprisingly found that the actual visibility 70 of the traffic aid, in terms of clear and distinct detection thereof by motorists, is not appreciably reduced by the provision of non-skid portions of substantially lesser high

light reflectivity on the whole marking surface, provided that the portion or portions having non-skid properties do not cover more than fifty percent of the area of said marking surface and that edge portions having high light reflectivity surfaces will uninterruptedly extend lengthwise the marking. As a matter of fact, the actual visibility, when considered as above, is apparently due to sharp reflectivity and color contrast with adjacent conventional roadway rather than amount of reflected radiations.

It has been further found that a surprising improvement of safe traffic and control of vehicles is attained by providing a marked road with a traffic aid having a compound surface as above, provided that at least twenty percent about of said surface of the marked area will possess non-skid properties.

These and other objects and advantages of the invention are in part obvious and in part will be made apparent as this description proceeds, and the features which are believed to be new and characteristic of the invention are in particular set forth in the appended claims. The invention itself, however, will be best understood from the following detailed description of preferred forms of embodiment thereof, when taken in conjunction with the accompanying drawings, forming an essential component of this disclosure, and wherein:

FIGURE 1 is a diagrammatical perspective fragmentary view of a marked road according to first embodiment of the invention;

FIGURE 2 perspectively and diagrammatically illustrates how the compound strip material components can be preformed and assembled;

FIGURE 3 similarly illustrates a marked road according to a modified embodiment of the invention;

FIGURE 4 is a perspective exploded view of the compound material of FIG. 3; and

FIGURE 5 illustrates a further embodiment of the invention.

Referring more particularly to the drawings, FIG. 1 shows a specific method of forming and applying a road marking compound material to a road surface S to actuate a centre or a track-dividing line, for example, or other sign having a given transverse dimension  $W_1$  for visibility.

According to current knowledge, such transverse dimension  $W_1$  is however a great deal larger than the size which might theoretically give the required visibility, i.e. the ability of reflecting the desired amount of light, provided that the sign has a clean, smooth and undamaged upper face. Adverse weather and lighting conditions are obviously to be taken into account in dimensioning such traffic regulation signs.

From another standpoint of view, however, there is a tendency to limit such transverse dimension within certain limits, six inches for example, because the currently elasto-plastic marking material have a more or less skidding upper face, on which vehicles' tires may easily skid with consequent prejudice of safety. It is known that a road marking material is as much visible and light-reflecting as it is smooth and skidding. Smoothness of the light-reflecting upper face of such materials is also critical for preventing said face to become readily dirty and dark, and therefore poorly visible.

By dividing the whole transverse dimension  $W_1$  of the sign means total surface, which will be hereby and in the appended claims defined as "marked area," in parts relatively coarse and non-skid and of relatively low visibility, and in parts of high reflectivity, said latter parts being adjacent to the marked area side edges, provided that the area of latter is at least fifty percent of the whole marked area, it has been found that the actual visibility of the sign will not substantially be prejudiced. It has been found that, at eyesight, clear visibility of such signs is essentially dependent on clear visibility of the side edge portions thereof.

Now, it might be assumed that the centre portion  $W_2$  wide of the marked area is not essential for improving

the visibility of the whole sign and, therefore, such centre portion  $W_2$  wide may be advantageously made such to possess improved non-skidding properties, essentially as an uncovered conventional road surface is. In addition, it might be assumed that the whole width  $W_1$  of the marking material may be increased with respect to the width of conventional elasto-plastic marking strips, as a consequence of the provision of the non-skid part  $W_2$  wide thereinto, the limit of such increment being given by the width of the portions designed for high light-reflection, individually considered.

According to what above,  $W_2$  is from 33 to 50 percent of  $W_1$ , and  $W_1$  is of four inches or above, according to the size and importance and average traffic speed of the marked highway, according to current art of road marking, a  $W_1$  width over six inches being however preferred.

The compound strip of FIG. 1 consists of a first base strip 10 of high reflectivity material, lengthwise recessed at 12, and of a strip 14 of material having non-skid properties, seated into and firmly secured in the recessed portion of the base strip.

According to FIG. 3, the base strip 20 has recessed portions 22 (FIG. 4) evenly spaced from the lateral edges thereof and wherein flat pieces 24 of non-skid properties possessing material are seated and secured in said recesses. Length L of individual pieces 24 may be comprised between 10 to 50 millimeters and the interval  $I_1$  therebetween may be comprised between 20 and 100 millimeters.

According to FIG. 5 two parallel longitudinal rows of pieces 34 spaced from each other and from the lateral edges of base strip 30 are provided for imparting non-skid properties to the traffic aid, the number of such row and the dimensions of the pieces being matter of choice, provided that a firm connection of said pieces to said base strip is ensured to resist to traffic and to wear and shearing forces induced thereby.

Some examples of formulations and of compositions of components will be described hereinbelow for best understanding of the invention and of the differing modes for carrying out same.

#### Example 1

This example illustrates formulations and combinations particularly adapted for producing a compound marking material the type shown in FIG. 1, which includes two components, namely a first high reflectivity component and a second non-skid component. The respective compositions' contents, expressed in terms of weight, will be indicated under "H-R" (for High Reflectivity) and "N-S" (for Non-Skid), respectively:

|    | Content                                                                                                               | H-R   | N-S   |
|----|-----------------------------------------------------------------------------------------------------------------------|-------|-------|
| 55 | Butadiene-acrylonitrile copolymer, having 38% acrylonitrile (acrylonitrile rubber "Chemigum No. 3," by Goodyear)..... | 20    | 20    |
| 56 | Maleic modified polyvinyl-chloroacetate copolymer ("Vinilite VMCH" by Union Carbide).....                             | 40    | 40    |
| 57 | Micromized calcium carbonate.....                                                                                     | 25    | ..... |
| 58 | Talcum 0000.....                                                                                                      | 25    | 50    |
| 59 | Zirconium oxide (average diameter .5 mils).....                                                                       | ..... | ..... |

65 The above compositions had been worked into the desired strip form preferably at 150° C. The components had been juxtaposed at 90° C. and the adhesive binding thereof had been attained upon the adhesive nature of such components, without making use of glues or other binding agents.

70 It will be noted that the "H-R" and "H-S" compositions differ from each other as the fillers thereof are concerned. The zirconium oxide, which may be substituted by similarly granulated quartz, imparts to the material the desired non-skid properties.

*Example 2*

A marking material for providing a marked road of the type shown in FIGS. 3 and 5 have been produced from the following compositions, by weight:

High reflectivity base strip component:

|                                                     |    |
|-----------------------------------------------------|----|
| Butadiene-acrylonitrile copolymer, having 38%       |    |
| acrylonitrile                                       | 12 |
| Maleic modified polyvinyl chloro-acetate co-polymer | 37 |
| Titanium dioxide (rutile)                           | 20 |
| Kaolin 0000                                         | 25 |
| Micromized calcium carbonate                        | 28 |

Five parts of a suitable plastifier, such as a coumaronic resin, can be added. The compound is processed and laminated in strip form at 150° C.

Non-skid components:

|                                                                               |     |
|-------------------------------------------------------------------------------|-----|
| Polychloroprene (such as "Neoprene WHV" by Dupont)                            | 25  |
| Isobutylene including 2.2% polyisoprene (such as "Butyl Rubber 402" by Shell) | 10  |
| Butadiene-acrylonitrile copolymer, having 38% acrylonitrile                   | 90  |
| Alkyl-acryl-phenol (such as "Vinstay V" by Goodyear)                          | 1   |
| Titanium dioxide                                                              | 80  |
| Sand                                                                          | 350 |
| Talcum A                                                                      | 200 |
| Quartz (average diameter .5 mils)                                             | 300 |

The compound has been processed and laminated at 90° C., and the desired pieces have been cut therefrom. Such pieces have been applied and secured to the base strip component, at 90° C., by making use of a glue consisting of

Glue:

|                                                                                       |    |
|---------------------------------------------------------------------------------------|----|
| 85% styrene polymer-15% butadiene polymer, such as "Marben 8000 A" by Marbon Chemical | 5  |
| Clear natural rubber                                                                  | 5  |
| Benzol                                                                                | 50 |
| Dichloroethane                                                                        | 40 |

While the invention has been described and shown in few forms of embodiment thereof, it is obvious that the invention itself is not limited to the very details shown, and that further modifications and variations might be made thereto, according to the art.

What is claimed is:

1. A marked road, comprising in combination, a road-

way surface for vehicles; a first strip of road marking tape having relatively low non-skid properties and high light reflectivity joined to the upper face of said roadway surface; and another strip formed of a material having non-skid properties and a lesser light reflectivity than said first strip of road marking tape and having a lesser width than said first strip extending in longitudinal direction and adhered to said first strip equally spaced from the lateral edges thereof so as to provide together with said first strip a composite surface formed of two spaced edge portions of said first strip of road marking tape having relatively low non-skid properties and high light reflectivity and of said other strip forming a center portion having non-skid properties and a lesser light reflectivity interposed between said two spaced edge portions of said first strip.

2. A marked road according to claim 1, wherein the width of said another strip is from one third to one half of the width of said first strip.

3. A marked road, comprising in combination, a roadway surface for vehicles; a first strip of road marking tape having relatively low non-skid properties and high light reflectivity adhesively joined to the upper face of said roadway surface; and strip components of a material having non-skid properties and a lesser light reflectivity than said first strip of road marking tape, said strip components being evenly spaced from each other and from the lateral edges of said first strip and adhered to said strip so as to provide together with said first strip a composite surface, longitudinally and laterally spaced portions of said first strip of road marking tape having high reflectivity and other portions spaced from said edges and having non-skid properties.

4. A marked road according to claim 3, wherein sum of the area of said portions having non-skid properties consists from twenty percent to fifty percent of the area defined between said lateral edges of first strip.

5. A marked road according to claim 3, wherein said portions having non-skid properties are arranged in a row of spaced elements equally spaced from the lateral edges of said first strip.

**References Cited****UNITED STATES PATENTS**

|    |           |         |            |       |        |
|----|-----------|---------|------------|-------|--------|
| 45 | 2,225,496 | 12/1940 | Gethin     | ----- | 94—1.5 |
|    | 2,898,825 | 8/1959  | Walker     | ----- | 94—1.5 |
|    | 3,011,412 | 12/1961 | Harrington | ----- | 94—1.5 |
|    | 3,049,980 | 8/1962  | Gill       | ----- | 94—1.5 |

50 NILE C. BYERS, *Primary Examiner.*